

No. 729,281.

PATENTED MAY 26, 1903.

W. E. COYAN.

PROCESS OF MAKING STEEL CASTINGS.

APPLICATION FILED JAN. 17, 1903.

NO MODEL.



Fig. 1.



Fig. 2.

Inventor

Wm E. Coyan,

*Sandmeyer & Co.*

Attorneys

Witnesses:  
Wm A. Curand.

Frank G. Radelfinger.

## UNITED STATES PATENT OFFICE.

WILLIAM E. COYAN, OF HOMESTEAD, PENNSYLVANIA.

## PROCESS OF MAKING STEEL CASTINGS.

SPECIFICATION forming part of Letters Patent No. 729,281, dated May 26, 1903.

Application filed January 17, 1903. Serial No. 139,446. (No specimens.)

*To all whom it may concern:*

Be it known that I, WILLIAM E. COYAN, a citizen of the United States, residing at Homestead, in the county of Allegheny and State of Pennsylvania, have invented new and useful Improvements in Processes of Making Steel Castings, of which the following is a specification.

My invention relates to an improved process for reducing the porosity, crystalline structure, and brittleness of steel castings and reducing internal strains therein, thereby greatly strengthening them and improving their durability.

15 I have illustrated my invention as applied to the forming of castings for rolls; but it is equally well adapted for many other articles.

Many attempts have been made to increase the strength and life of cast-steel rolls, and 20 of the methods devised the most important is the process of first casting the rolls and then annealing them by first letting them cool and then slowly reheating them from forty-eight to seventy-two hours, thereby bringing 25 them up to a temperature of about 925° centigrade, after which the furnace is banked and the temperature held constant for about the length of time employed in reheating. This treatment gives good results, but adds greatly 30 to the cost of the rolls. To obtain equally good results at a decreased cost is an object of my invention.

The simple and novel method devised for accomplishing the object above set forth is 35 fully described and claimed in this specification and illustrated in the accompanying drawings, forming a part thereof, in which—

Figure 1 is a vertical longitudinal section of a mold with a cooling-pipe mounted therein 40 and containing a casting. Fig. 2 is a transverse section of the same.

The numeral 1 designates a mold for casting a hollow roll, and mounted in said mold to serve as a core and also as a means for internally chilling the casting is a pipe 2, surrounded by an external jacket 3, of asbestos or other non-inflammable and high-fusing material. The pipe 2 extends throughout the length of the mold 1 and is provided with 45 unions 4 on its free ends to enable it to be coupled at one end to a pipe 5, communicating with some source of cooling medium, either

liquid or gaseous, and at the other end to a waste-pipe 6.

In casting a roll the cooling medium, generally cold water, is first permitted to run through the pipe 2 to thoroughly cool it and the jacket 3 thereon. The molten metal is then poured into the mold 1 to form a casting 7, surrounding the pipe 2. The water is allowed to continue running through the pipe 2 until the part surrounding the pipe and adjacent to it becomes sufficiently cool to stand alone, after which the pipe 2 is uncoupled from the pipes 5 and 6 and withdrawn and a stream of the cooling medium played into the resulting aperture in the casting 7 made by the pipe 2. The stream is continued until the center of the casting 7 becomes chilled; but the outer portion still retains sufficient heat to reheat the chilled portion after the stream is discontinued. To give a more definite idea as to the temperatures employed, it may be stated that immediately after casting the roll the temperature of the whole mass is uniform and approximately 1200° centigrade. By the chilling process the temperature of the center portion of the roll surrounding the core is then reduced to about 700° centigrade, when the cooling is discontinued. The excess of heat of the outside portion of the roll over the center will then reheat the center until the whole mass again attains a substantially uniform temperature in the neighborhood of 900° to 925° centigrade, when the cooling proceeds uninterrupted. Should the cooling be continued until the casting 7 is completely cooled, I find that the resulting product would be too brittle; but the stopping of the cooling while heat enough remains in the outer portion of the casting to reheat the interior produces the annealing effect so much desired and decreases the internal strains, besides reducing the crystalline structure and porosity of the resulting roll, and therefore the brittleness.

While I have mentioned water as the cooling medium employed, I may use any of the well-known liquids or gases commonly used for chilling steel, such as brine, oil, compressed air, &c.

Many of the results of my method may be attained by an abbreviated method which consists in using a mold having a core-pipe

mounted therein having no jacket thereon, then starting the flow of cooling medium through the core before pouring in any of the molten metal, then pouring in the molten metal while the flow continues, and continuing the flow of cooling medium until the interior of the casting has become chilled, but heat enough remains in the outer portions of the castings to reheat the interior.

10 Having thus described my invention, what I claim as new, and desire to secure by Letters Patent, is—

15 1. The process of forming steel castings to increase their tenacity and reduce their porosity, which consists in mounting a pipe in a mold, then running a cooling medium through said pipe, then pouring molten metal into said mold and permitting the running of the cooling medium until the casting is cold enough to stand alone, then withdrawing said pipe, then playing a stream of said cooling medium into the resulting aperture in the casting to cool the interior of the casting, and then discontinuing said stream to permit the heat in the outer portion of the casting to reheat the cooled inner portion, substantially as described.

20 2. The process of forming steel castings, which consists in forming a mold for a casting and mounting a pipe in said mold to serve as a core, then pouring molten metal into said mold to surround said pipe, then running a cooling medium through said pipe until said casting will stand alone after said pipe has been withdrawn, then withdrawing said pipe, then playing a stream of cooling medium into the resulting aperture until the adjacent portion of said casting has become cool but heat enough remains in the casting 40 to reheat said cooled portion, substantially as described.

25 3. The process of forming steel castings which consists in mounting a pipe in a mold for forming a casting, said pipe being protected by suitable means to keep it from being burned up by the molten metal, then running molten metal into said mold and around said pipe, then running a cooling medium through said pipe until said casting will stand alone, then withdrawing said pipe and playing a stream of cooling medium into the resulting aperture until the adjacent portion of the casting has become cooled, but the outer portion still remains hot, and then discontinuing said stream to permit the remaining heat in said casting to reheat said cooled portion, substantially as and for the purpose set forth.

4. A method of forming a steel casting, which 60 consists in providing a mold for said casting having a hollow core therein, then pouring molten steel into said mold to surround said core, and then passing a cooling medium through said core until the adjacent parts of the casting have been cooled but the exterior parts still retain heat enough to reheat said cooled portion, then stopping the passage of

70 said cooling medium to permit the chilled portion to be reheated several hundred degrees by the excess of heat in the exterior of the casting to reduce the porosity of the resulting roll, substantially as described.

5. A method of forming steel castings which consists in providing a mold for a casting with a hollow core located centrally therein, then 75 pouring molten metal into said mold, then passing a cooling medium through said core until the casting will stand alone, and then removing said core and playing a stream of cooling medium in the resulting aperture to 80 cool the adjacent parts but leave the outer portion hot, then discontinuing the playing of said stream and permitting the excess of heat in the exterior portion of the casting to reheat the chilled interior to reduce the porosity of the casting, substantially as described.

6. The method of forming steel castings, which consists in providing a mold having a core therein, pouring molten metal into said 90 mold and permitting it to cool until said casting will stand alone, and then removing said core and playing a stream of cooling medium into the resulting aperture to cool the interior of said casting but not the exterior which retains heat enough to draw the temper of the cooled interior portion, substantially as described.

7. A method of forming steel castings, which consists in providing a mold for said casting 100 with a hollow core, then starting the flow of a cooling medium through said core, then pouring the molten metal into said mold while the flow of cooling medium continues, and continuing the flow of the cooling medium 105 until the center of the casting has become chilled but heat enough remains in the exterior portion to reheat the interior, then discontinuing the flow of said cooling medium to permit the chilled portion to be reheated 110 by the excess of heat in the exterior portion to produce an annealing effect and decrease the porosity and strains in the resulting casting, substantially as and for the purpose set forth.

8. A method of forming castings, which consists in providing the mold therefor with a non-communicating internal hollow metal core of a temperature below that of the surrounding mold, then pouring the molten 120 metal in the mold to surround said core, then maintaining a low temperature in said core by passing a cooling medium therethrough to reduce the temperature of the casting thereof to a greater degree than that of the exterior of said casting, and then discontinuing the flow of the cooling medium to permit the heat at the exterior to gradually extend to and raise the temperature of that part surrounding the core, substantially as described.

9. A method of forming castings, which consists in providing a mold therefor, with a non-communicating internal hollow metal core the temperature of which is maintained at a low

degree by passing a cooling medium there-  
through, then pouring the metal in the mold  
to surround said core to decrease the tempera-  
ture of the metal surrounding the core to a  
greater degree than that at and toward the  
exterior portion thereof, and then discontinu-  
ing the flow of cooling medium through the  
core to permit the heat at and adjacent to the  
exterior to gradually raise the temperature

at that part surrounding the core, substan- 10  
tially as described.

In testimony whereof I have hereunto set  
my hand in presence of two subscribing wit-  
nesses.

WILLIAM E. COYAN.

Witnesses:

WM. H. C. SMITH,  
J. CLYDE MILLER.